# EUROPEAN PATENT APPLICATION

(11) **EP 3 495 459 A1**
(43) Date of publication of application: **12.06.2019**
(21) Application number: 16190996.5
(22) Date of filing: 28.09.2016
(51) Int. Cl.: C10L 5/04, C10L 10/08

(54) **THE COMPOSITION OF A LIQUID LUBRICANT AND ITS USE**

(30) Priority: 31.07.2015 PL 41336615
(71) Applicant: Skotniki, Wieslaw, 68-200 Zary (PL)
(72) Inventor: Skotniki, Wieslaw, 68-200 Zary (PL)
(74) Representative: Godlewski, Piotr

(57) **Abstract**

The subject of the invention is composition of a liquid lubricant being a suspension made based on vegetable oils or modified animal fats, additionally comprising solid lubricants and ancillary substances, such as: suspension stabilisers, pigment, paraffin dispersants, as well as its use in boilers fed by screw conveyors, fired with black coal.

## Description

The subject of the present invention is the composition of a liquid lubricant along with its use. More precisely, the solution relates the composition of a liquid lubricant for boilers fed by screw conveyors, fired with black coal.

In the state of the art there is no information about the existence and use of liquid lubricants for coal and for screw conveyors in boilers fired with black coal, whose primary purpose is to reduce the friction existing when moving lumps (pieces) of coal by means of a screw conveyor, piston conveyor or any other conveyor where the phenomenon of friction occurs.

The lubricants for boilers described in the state of the art are only used to improve the combustion, reduce the emission of harmful substances and prevent corrosion.

Document DE 4424090A1 discloses an aqueous solution of alkaline earth compounds combined with an aqueous solution of Fe, Ca, Mg, K salts used to improve the combustion of coal and additionally preventing corrosion and reducing the generation of SOx and NOx.

On the other hand, document US7341447 discloses a method for reducing the harmful impact of substances originating from the combustion of hydrocarbon fuels by lubricating the boiler with a lubricant comprising oils and additional substances, comprising at least one organosulfur compound or at least one organophosphorus compound, or both, and at least one source of manganese, wherein the lubricant being added to the boiler separately from the fuel.

On the other hand, document US4842617 discloses a method for improving the combustion of fuel in furnaces by adding a magnesium compound in the form of a fine-grained mixture. This addition also reduces corrosion.

Document US4262610 discloses a method of reducing the emission of sulphur in furnaces fired with coal, which comprises adding a fine-grained form of calcium oxide along with fuel.

Document GB1360750 discloses a method of treating a briquette made of coal or a mixture comprising coal and coke by pressing in a temperature of 400-540°C, wherein the briquette is submersed in a temperature of 250-450°C in an aqueous solution of the cement. Such treating of the briquette causes its better combustion.

However, in boilers fed by screw conveyors and fired with black coal, hereinafter referred to as boilers, no additional technical solutions are used to minimise the friction between coal and the screw conveyor, as well as between the lumps of coal. As a result of this, the friction in the screw conveyor causes damage to the surface of the screw and the inner surface of the conveyor, as well as damage to the mechanical protection element (the locking pin). The moving of coal in the conveyor without using a liquid lubricant for boilers fed by screw conveyors, fired with black coal results in the generation of uncomfortable noise. Additionally, the friction causes significant use of electric energy and the harmful results of engaging electric devices, in particular the contacts of the relays as well as the brushes and the rotor of the motor.

Therefore, the purpose of the invention is to provide a liquid lubricant for boilers fed by screw conveyors, fired with black coal, which would solve the above-mentioned problems, and would therefore result in:
- decreasing the friction between coal and the screw conveyor as well as between the lumps of coal,
- decreasing the wear of the mechanical elements of the conveyor, its drive and the means of protection,
- reducing the uncomfortable noise caused by the screw crushing the coal,
- decreasing the consumption of electric energy consumed by the motor driving the screw,
- decreasing the wear of the contacts of the controller's relays and the elements of the driving motor, and
- decreasing the corrosion of the conveyor's elements and the combustion chamber caused by volatile sulphur compounds.

Additionally, the use of a liquid lubricant for boilers fed by screw conveyors, fired with black coal according to the invention allows gaining additional ecological benefits, including the reduction of the emission of carbon dioxide into the atmosphere by energy producers and a slight reduction of the sulphur compounds emitted as a result of the combustion process in boilers.

The object of the invention is the composition of a lubricant, characterised in that it is a suspension made based on vegetable oils or modified animal fats, additionally comprising solid lubricants and ancillary substances.

Preferably, the solid lubricants are solid paraffins, stearin, solid fats, fatty acids salt of metals from first and second group.

Preferably, the ancillary substances are suspension stabilisers, pigments, paraffin dispersants.

Preferably, the composition can additionally comprise calcium or/and magnesium salts of organic and inorganic acids.

Preferably, the composition is characterised in that it exists in a liquid form and its density ranges between 900 kg/m³ and 1000 kg/m³.

Preferably, the composition comprises vegetable fats or modified liquid animal fats amounting from 60 to 90 wt%, stearin in amount of 2-5 wt%, soft paraffins in amount of 2.5-7 wt%, hard paraffins in amount of 2.5-7 wt%, calcium stearate or calcium palmitate in amount of 5-15 wt%, calcium or magnesium carbonate in amount of 1-10 wt%, suspension stabilisers, thixotropic agents, dyes and pigments, other ancillary substances in a total amount up to 5 wt%.

Preferably, the composition comprises vegetable oils amounting between 60 and 90 wt%, stearin amounting from 1 to 5 wt%, soft paraffins amounting from 2.5 wt% to 7.5 wt%, hard paraffins amounting from 2.5 wt% to 7.5 wt%, calcium stearate from between 3 to 15 wt%, ancillary agents amounting to up to 5 wt%.

Another object of the invention is the use of the composition described above in boilers fed by screw conveyors, fired with black coal.

Preferably, the lubricant is added directly and centrally atop the heap of coal in the storage tank.

The invention will be further illustrated by use of non-limiting embodiments.

### Example 1

The composition of liquid lubricant for boilers fed by screw conveyors, fired with black coal is a suspension of density between 900 kg/m³ and 1000 kg/m³, made based on vegetable oils or modified animal fats, additionally comprising solid lubricants such as: solid paraffins, stearin, solid fats, fatty acids salt of metals from first and second group, as well as ancillary substances such as: suspension stabilisers, pigment, paraffin dispersants.

The quantities of the composition's components are presented below.

**Table 1**

| Chemical name | Amount (wt%) |
|---|---|
| vegetable oil | 60-90 |
| stearin | 1-5 |
| soft paraffins | 2.5-7.5 |
| hard paraffins | 2.5-7.5 |
| calcium stearate | 3-15 |
| ancillary agents | up to 5 |

### Example 2

The composition of liquid lubricant for boilers fed by screw conveyors, fired with black coal is a suspension of density between 900 kg/m³ and 1000 kg/m³, made based on vegetable oils or modified animal fats, comprising solid lubricants such as: solid paraffins, stearin, solid fats, fatty acids salt of metals from first and second group, as well as ancillary substances such as: suspension stabilisers, pigment, paraffin dispersants, and it can also additionally comprise the calcium or/and magnesium salts of organic and inorganic acids, added in order to reduce the corrosion of the elements of the screw conveyor, caused primarily by sulphur compounds.

The quantities of the composition's components are presented below.

**Table 2**

| Name of the substance | Amount (wt%) |
|---|---|
| vegetable oil or modified liquid animal fat | 60-90 |
| stearin | 2-5 |
| soft paraffins | 2.5-7.5 |
| hard paraffins | 2.5-7.5 |
| calcium stearate or calcium palmitate | 5-15 |
| calcium or magnesium carbonate | 1-10 |
| suspension stabilisers, thixotropic agents, dyes and pigments, other ancillary substances | up to 5 |

The liquid lubricant for boilers fed by screw conveyors, fired with black coal is used by adding a portion of the lubricant directly and centrally atop the heap of coal in the storage tank.

## Claims

1. The composition of a lubricant, **characterised in that** it is a suspension made based on vegetable oils or modified animal fats, additionally comprising solid lubricants and ancillary substances.

2. The composition according to claim 1, **characterised in that** the solid lubricants are solid paraffins, stearin, solid fats, fatty acids salt of metals from first and second group.

3. The composition according to any of the above claims, **characterised in that** the ancillary substances are suspension stabilisers, pigments, paraffin dispersants.

4. The composition according to any of the above claims, **characterised in that** it can additionally comprises calcium or/and magnesium salts of organic and inorganic acids.

5. The composition according to any of the above claims, **characterised in that** it exists in a liquid form and its density ranges between 900 kg/m³ and 1000 kg/m³.

6. The composition according to any of the above claims, **characterised in that** it comprises vegetable fats or modified liquid animal fats amounting from 60 to 90 wt%, stearin in amount of 2-5 wt%, soft paraffins in amount of 2.5-7 wt%, hard paraffins in amount of 2.5-7 wt%, calcium stearate or calcium palmitate in amount of 5-15 wt%, calcium or magnesium carbonate in amount of 1-10 wt%, suspension stabilisers, thixotropic agents, dyes and pigments, other ancillary substances in total amount up to 5 wt%.

7. The composition according to any claim from 1 to 5, **characterised in that** it comprises vegetable fats amounting from 60 to 90 wt%, stearin amounting from 1 to 5 wt%, soft paraffins amounting from 2.5 wt% to 7.5 wt%, hard paraffins amounting from 2.5 wt% to 7.5 wt%, calcium stearate amounting from 3 to 15 wt%, ancillary agents amounting up to 5 wt%.

8. The use of the composition of a lubricant according to claims 1-7 in boilers fed by screw conveyors, fired with black coal.

9. The use of the composition of a lubricant according to claim 8, **characterised in that** the lubricant is added directly and centrally atop the heap of coal in the storage tank.
